

## UNITED STATES PATENT OFFICE

1,972,502

## METHOD OF FINISHING WOOD

Frank Tuchfarber, deceased, late of Cincinnati, Ohio, by William K. Divers, administrator, Cincinnati, Ohio, assignor, by mesne assignments, to R. W. Callaway, New York, N. Y. and Alan N. Mann, Scarsdale, N. Y., as joint trustees

No Drawing. Application December 13, 1932,  
Serial No. 646,998

7 Claims. (Cl. 91—68)

The invention herein involved relates to a new method of treating wood, or other material having fibrous surfaces, as part of the finishing operation. This treatment is particularly aimed to 5 producing surfaces of great beauty but in addition when applied (particularly in preferred form) to wooden members used as sounding boards in musical instruments as, for example, violins or the sounding boards of pianos, it produces an extraordinary fine resonance. It is recognized 10 that natural wood when dry has a better resonance than the same wood finished in ordinary ways, but a finish is necessary to preserve the wood and prevent undue penetration of moisture. Finishes applied using the invention of this application 15 preserve the resonance and tone quality to a marked degree.

In its preferred embodiment, the invention is a very simple one and consists in formulating a 20 combined solution and suspension of gluten and gamboge in water, which is applied to the clean, smooth surface of the natural wood and allowed to dry. The wood should preferably be "in the white" and not previously treated. This first application 25 results in the formation on the surface of the wood of a muddy unattractive layer which completely or substantially hides the surface of the material. This, however, is followed with coatings of usual commercial varnish, or lacquer, 30 or other like film-forming material made with an organic solvent. Immediately after the first coating of this finishing material is put on, a distinct change in the surface is observed, and within a few moments there is obtained a beautiful 35 lumenous effect giving richness and clearness to each detail of the grain markings. Apparently this result is due to the fact that the preliminary treatment coats the surface of the wood with a layer of minute particles of substantially colloidal 40 size, and these are gradually dissolved in the subsequent layers of finish. Where gamboge is employed, the color seems to blend through into each successive layer of finishing material, making a highly refractive film which seems to bring 45 out, through selective action, all the beauty of the grain markings, emphasizing the character of each species of wood. As might be expected, the effect is particularly beautiful on light, highly grained woods such as maple and birch, yet its 50 effect on such woods as mahogany and walnut is strikingly noticeable.

Apparently the preliminary treatment is such that there is very little penetration, for the solid material tends to stay on the surface and 55 acts to prevent the subsequent penetration of the

finish even though this solid material is dissolved in the finishing coat. According to observations made when the coating is applied, the protective qualities of the finish on wood are probably a function of the adhesion developed between the 60 fibers of the wood and the protective film. Under the layer of solid particles formed according to the present invention, the preliminary coating described forms a continuous resistant film which, as the gradual solution of the particles takes 65 place, becomes an integral part of the subsequent coats, so that the several layers are welded into a protective body which is very effective as a moisture retardant and likewise assists in holding the film mass in the desired semi-fluid state essential 70 to a permanent, durable finish. Because of this action this treatment is in some cases valuable as a base for pigmented film forming materials, as for example in the case of coating very porous bodies such as pressed board made of vegetable 75 fibers.

As stated above, the preferred embodiment of the invention utilizes gluten and gamboge. Gamboge is a gum resin with a part soluble in water and a resinous part which is insoluble. The gum 80 which is dissolved in water seems to serve as a dispersing agent to assist in maintaining the insoluble resin in suspension. The gluten also appears to act as a dispersing agent, smoothing 85 the product and making it easier to apply and it may act somewhat to plug the pores of the wood and prevent undue penetration.

It will readily be seen that numerous materials can be used as more or less equivalent to the preferred ingredients; for example, myrrh is a gum 90 resin having qualities somewhat similar to gamboge but without including the characteristic yellow color, and myrrh gives quite similar results to gamboge. Also synthetic gum resins can readily be produced by grinding with water in a 95 colloid mill a natural resin such as rosin, or a synthetic resin such as a phenolic resin while in the intermediate or so-called soluble state, with a gum such as gum arabic or tragacanth. In like manner, there are various recognized equivalents 100 for gluten which will serve as dispersing agents, such for example as casein, various vegetable proteins or soaps, and in some cases the gum alone will serve without this added ingredient.

The preparation of the preliminary coating material is very simple and this material is also very inexpensive, as relatively small amounts of solids are used in the water and the prepared product has remarkable covering power. Even though water is used, there is a surprisingly small 110

raising of the grain or swelling of the surface fibers, especially when the coating is applied with the grain with rapid, even strokes, or preferably by spraying. A particularly notable characteristic of the composition is its rapid drying, making it possible to apply the first coat of finish within an hour after the preliminary treatment. The usual time is allowed to lapse between subsequent applications of the finish, and the surface may or 10 may not be rubbed down between coats, according to the type of finish desired. However, it will be found that fewer coats of the finishing material are needed than is ordinarily the case.

The method in which the preliminary treating 15 material is prepared can readily be understood from the following example, though this is given only by way of example and the proportions used may be modified widely:

A medium sized teaspoonful of gluten flour is 20 placed in a cup. To this is added a teaspoonful of clean water. The two are stirred together into a smooth paste and there is then added an ounce or two of lukewarm water which is likewise stirred in. The thin paste thus formed is then 25 added to about two gallons of lukewarm water and slowly boiled until the volume is reduced to one gallon.

If these directions are followed, it will insure 30 a thorough cooking of the gluten but it is to be understood that they are not positive limitations.

The gallon of material thus prepared is cooled and filtered through a coarse filtering medium and care should be taken to preserve this solution against souring.

35 One and one-half ounces of powdered gamboge are mixed with six ounces of clean water and thoroughly agitated. After allowing the two to stand together for about 24 hours, preferably with frequent agitation, the material is filtered 40 through a coarse filter, such as a linen or muslin cloth, which will remove suspended particles of excessive size; but this filtering step may not be necessary if the gamboge has been reduced to a sufficiently fine powder in the first instance.

45 To make the complete preliminary coating material, the gluten water and gamboge suspension may be mixed in equal volumes. These proportions are intended only as a guide to the practice of the invention and are subject to wide variation; 50 for example, the materials may be mixed in proportions ranging up to 3:1, with either of the materials forming the greater proportion. As stated above, under some circumstances the gluten may be entirely omitted, but ordinarily its 55 presence improves the result. The complete coating material improves if allowed to stand for a number of hours before using.

The preliminary coating material is preferably applied quite rapidly over the surface of the clean, 60 smooth wood. A brush may be used or a small pad, such for example, as may be made by wrapping a rubber sponge in a muslin cloth. This pad should be moist but not wet, and to get the best results the wood should be gone over only once and the material should be applied with the grain rather than across it. If desired, a spray 65 gum may be used for application. As has already been stated, the preliminary coating dries very rapidly and as soon as it has dried the finishing 70 coats of varnish or lacquer can be applied with a brush or in other manners known to those skilled in the art of finishing wood.

75 The invention herein described when applied to wood and other fibrous surfaces according to the usual methods of one familiar with the art

of finishing, results in the formation of finished surfaces of superior quality as regards both beauty and utility with marked economy in both time and cost of application. Further, as has already been stated, when this finish is used in connection with musical instruments it produces musical sounding boards rich and mellow in tone with resonant carrying qualities, presumably because the film of the coating layers is held on the surface, permitting the wood to retain its natural vibratory characteristics.

35

What is claimed is:

1. The method of finishing fibrous surfaces which comprises applying to such a surface a colloidal suspension in water of an undissolved resinous material insoluble in water but soluble in organic solvents, permitting the resulting coating to dry without substantially softening the resinous ingredient, and applying a film forming compound comprising an organic solvent adapted to dissolve said resin.

90

2. The method of finishing fibrous surfaces which comprises applying to such a surface a watery suspension comprising an undissolved resinous material insoluble in water but soluble in organic solvents, and an organic dispersing agent, permitting the resulting coating to dry without substantially softening the resinous ingredient and applying a film-forming material comprising an organic solvent adapted to dissolve said resin.

100

3. The method of finishing fibrous surfaces which comprises applying to such a surface a watery suspension comprising an undissolved resinous material insoluble in water, a water-soluble gum and an organic dispersing agent, permitting the resulting coating to dry without substantially softening the resinous ingredient and applying a film-forming material comprising an organic solvent adapted to dissolve said resinous material.

110

4. The method of finishing fibrous surfaces which comprises applying to such a surface a watery suspension of an undissolved gum resin and an organic dispersing agent, permitting the resulting coating to dry without substantially softening said gum resin and applying a film-forming material comprising an organic solvent adapted to dissolve said resin.

115

5. The method of finishing fibrous surfaces which comprises applying to such a surface a watery suspension of gamboge and gluten, permitting the resulting coating to dry, and applying a film-forming material comprising an organic solvent adapted to dissolve the non-water soluble portions of the gamboge.

125

6. As a new article of manufacture, a fibrous board-like body having a protective film firmly adhering to the surface thereof without extensive penetration, such film resulting from the solution in situ of a layer of distinct particles of substantially colloidal size of a soluble resin by an ingredient of a finishing film-forming material applied thereto.

130

7. As a new article of manufacture, a wooden sounding board having a protective film firmly adhering to the surface thereof without extensive penetration, such film resulting from the solution in situ by an ingredient of a film forming material applied thereto, of a layer of distinct particles of substantially colloidal size of a resin soluble in organic solvents but insoluble in water which is present on the surface of such board in conjunction with an organic dispersing material.

135

140

145